

I. J. VOLKOMMER.  
MAKING METALLIC OXIDS.  
APPLICATION FILED DEC. 26, 1916.

1,300,522.

Patented Apr. 15, 1919.



**WITNESSES**

W. T. Holman  
John Bailey Brown

**INVENTOR**

Theodore J. Vollkommer  
By Frank W. Winter  
HIS ATTORNEY

# UNITED STATES PATENT OFFICE.

THEODORE J. VOLLKOMMER, OF PITTSBURGH, PENNSYLVANIA.

## MAKING METALLIC OXIDS.

1,300,522.

Specification of Letters Patent. Patented Apr. 15, 1919.

Application filed December 26, 1916. Serial No. 138,953.

*To all whom it may concern:*

Be it known that I, THEODORE J. VOLLKOMMER, a resident of Pittsburgh, in the county of Allegheny and State of Pennsylvania, have invented a new and useful Improvement in Making Metallic Oxids, of which the following is a specification.

This invention relates to a method and apparatus for producing metallic oxids, such for instance as the oxids of lead, tin, 10 antimony, and of other metals.

The object of the invention is to provide for the production of such oxids more rapidly, with less labor, and of a finer and better 15 quality than as heretofore produced.

The essential features of the invention consists in maintaining a relatively shallow bath of the metal to be oxidized in molten condition upon a furnace hearth or bottom 20 which is porous or perforate so that an oxidizing gas, for instance air, can be made to pass through the bottom or hearth and through the bath of metal contained thereon, whereby the oxygen of the oxidizing gas 25 will oxidize said metal; and preferably at the same time directing blasts of the oxidizing gas, such as air, against the surface of the molten bath on the hearth, whereby further metal is oxidized, or in the event 30 that the oxidizing gas coming through the body of the metal produces only a partial oxidation, that introduced above the molten bath will fully oxidize the same. And further it is proposed to heat the oxidizing gas 35 before applying it to the metal.

The accompanying drawing is a vertical section, somewhat diagrammatic, through a furnace suitable for carrying out the invention.

As shown in the drawings, a preferred 40 form of the furnace comprises a suitable hearth or bottom 1 for the furnace chamber 2 which is formed by said bottom and the side walls 3 and roof or top 4. This entire furnace is surrounded by a chamber 5 formed by intermediate side walls 6, top or roof 7, and bottom 8, and this in turn is surrounded by another chamber 9 formed by the same bottom 8, exterior side walls 10 45 and a roof 11. The hearth or bottom 1 rests upon suitable supports 12 in a manner such that the space underneath the bottom 1 is in communication with the chamber 5, which chamber is adapted to have supplied thereto an oxidizing gas, such as air, through a blast pipe 14 which will be connected to

any suitable air source. The hearth or bottom 1 is a porous or perforate plate. It can be formed from any suitable material, such as a filter plate, sufficiently porous to permit 60 gases to pass therethrough, or of even denser substances, but in the latter event will be provided with very small perforations to permit the gas to pass through the same, but not sufficiently large to permit molten 65 metal to escape therethrough. A layer or bath of metal 15 to be oxidized in molten condition, is shown on the hearth or bottom 1, and 16 indicates a series of small openings through the side walls 3 leading from 70 the exterior chamber 5 to the interior chamber 2, and preferably inclined, as shown, so as to direct the oxidizing gas against the surface of the molten metal. The chamber 9 which entirely surrounds the furnace, is 75 merely a preheating chamber, and has communicating therewith at suitable intervals around the furnace, burners 17, by means of which the furnace can be heated sufficiently to start the reaction or to maintain the reaction after starting. Generally, however, little or no additional heat is required after the reaction has started, as this reaction will furnish sufficient heat. The heating chamber 9 is connected through flue 18 to a suit- 80 able stack.

The oxids which are formed are drawn from the chamber 2 through a central top outlet 19 communicating with a lateral flue 20 leading to a suitable filter. At the upper 90 end of the vertical outlet 19 is a hopper or receptacle 21 controlled by a valve 22 through which the metal to be oxidized is fed to the furnace in suitable quantities.

In using this apparatus, the furnace is 95 heated by means of the burners 17, a sufficient amount of metal to be oxidized being introduced into the chamber 2 from hopper 21 through valve 22, in sufficient quantity to form a thin shallow bath of molten metal 100 on the bottom 1. The oxidizing gas passes through pipe 14 into chamber 5, in which it is preheated and it then passes up through the porous bottom and also through the blast orifices 16. The oxidizing gas, passing 105 up through the porous bottom, percolates through the molten metal, converting it into an oxid. If the molten bath is sufficiently shallow, the oxidation will be complete, and in that event it is not essential that additional air be admitted through ports 16, but in case the molten bath is quite deep, the 110

oxidation within the bath will not be perfect, but various preliminary oxids will be formed, and in that event additional oxidizing gas coming through the blast openings 5 16 is necessary in order to complete the oxidation.

Actual use of the furnace in the manner described has demonstrated that the oxid which is formed is of very excellent quality, 10 10 being a pure oxid of the metal used, and in the form of a very light impalpable powder, which is carried by the air passing from chamber 2 through the outlet 19 and flue 20 to the filter. The oxidation takes place very 15 rapidly and no labor is necessary other than merely to supply the necessary amount of metal from time to time, all of the other actions taking place entirely automatically within the furnace.

20 Heretofore, such oxids have been produced almost entirely on an open hearth or furnace bottom by merely allowing the air to pass over the same, and scraping the film of oxid off the surface as rapidly as it forms.

25 This old process requires constant scraping of the surface, as otherwise the film will protect the unoxidized metal underneath. The oxid so formed is not, however, so pure or of so light and fine a texture as that formed 30 by the new method; and the scraping process frequently carries small particles of unoxidized metal with the oxid, resulting in trouble when the latter is used for such purposes as enameling, etc.

35 While I have described a form of my invention comprising a closed furnace with surrounding closed spaces, and air heated

by gas burners, and passed through the metal under pressure, I may use other forms of the apparatus, and other heating means. 40 My invention is therefore not to be limited to the exact forms shown.

What I claim is:—

1. An apparatus for producing oxids of metal comprising a furnace having a porous or perforate bottom and perforate side walls, a chamber surrounding said furnace and bottom, and means for introducing an oxidizing gas under pressure in said surrounding chamber. 45

2. An apparatus for producing oxids of metal comprising a furnace having a porous or perforate bottom and perforate side walls, a chamber surrounding said furnace and bottom, means for introducing an oxidizing gas under pressure in said surrounding chamber, and a heating chamber surrounding said furnace and provided with means for heating the entire furnace. 50

3. An apparatus for producing oxids of metal comprising a furnace having a porous or perforate bottom and perforate side walls, a chamber surrounding said furnace and bottom, means for introducing an oxidizing gas under pressure in said surrounding chamber, a charging hopper connected to the furnace, and an outlet flue for the oxids connected to said inner chamber. 55

In testimony whereof, I have hereunto set my hand.

THEODORE J. VOLLKOMMER.

Witnesses:

GLENN H. LERESCHE,  
A. E. JOHNSON.